

# United States Patent [19]

Randak et al.

[11] 3,784,418

[45] Jan. 8, 1974

[54] **PROCESS FOR THE MANUFACTURE OF COLD-ROLLED SHEETS FROM A RUST-RESISTANT, FERRITIC STEEL ALLOY CONTAINING CHROMIUM AND MOLYBDENUM**

[75] Inventors: **Alfred Randak; Karl Michel**, both of Huttental-Geisweid, Germany

[73] Assignee: **Stahlwerke Sudwestfalen AG**, Huttental-Geisweid, Germany

[22] Filed: Nov. 3, 1970

[21] Appl. No.: 86,610

[30] **Foreign Application Priority Data**

Nov. 3, 1969 Germany ..... P 19 55 026.6

[52] U.S. Cl. ..... 148/12

[51] Int. Cl. ..... C21d 9/48

[58] Field of Search ..... 148/12, 12.1, 12.3; 75/126 R

[56] **References Cited**

UNITED STATES PATENTS

|           |         |                         |          |
|-----------|---------|-------------------------|----------|
| 2,851,384 | 9/1958  | Waxweiler .....         | 148/12   |
| 3,067,072 | 12/1962 | Leffingwell et al. .... | 148/12   |
| 3,139,358 | 6/1964  | Graziano .....          | 148/12   |
| 3,490,956 | 1/1970  | Wilton .....            | 75/126 R |

Primary Examiner—W. W. Stallard

Attorney—Burgess, Dinklage & Sprung

[57] **ABSTRACT**

Cold-rolled strip and sheets are made from a special steel alloy containing chromium and molybdenum by subjecting hot-rolled strip formed from the alloy to multi-stage annealing at controlled temperatures and thereafter cold rolling and annealing after each cold rolling step.

**13 Claims, No Drawings**

**PROCESS FOR THE MANUFACTURE OF  
COLD-ROLLED SHEETS FROM A  
RUST-RESISTANT, FERRITIC STEEL ALLOY  
CONTAINING CHROMIUM AND MOLYBDENUM**

**BACKGROUND**

This invention relates to a process for the manufacture of cold-rolled strips and sheets from corrosion-resistant, ferritic chromium steel with molybdenum added, having improved deep drawing characteristics similar to austenitic steel.

Deep drawing ability is considered as one of the important criteria in judging flat products. In the case of fine sheets, the steels used consist substantially of unalloyed ferritic steels, ferritic chromium steels and austenitic chromium nickel steels.

The austenitic chromium nickel steels and the low-carbon unalloyed steels have excellent deep drawing characteristics, it being a rule that a reduction of the strength characteristics, especially the yield point, results in an improvement in deep drawing ability.

It is also known, however, that the mechanical-technological properties of flat sheet-like products are impaired by chromium alloying. Rust-resistant steels of the quality X 8 Cr 17 according to DIN Preliminary Standard 17440 have substantially poorer deep drawing ability than unalloyed steel types ("Blech" No. 11, 1965, page 627).

Although the above-mentioned X 8 Cr 17 grade of steel has a high corrosion resistance, it is necessary, where stronger corrosive attack is involved, to alloy about 1 percent molybdenum with the 17 percent chromium. This molybdenum content gives this steel an improved resistance to attack by reducing and chloride-containing corrosive media, with which it comes in contact, for example, when it is used in automobile parts exposed to road salt, industrial atmospheres, and the like. However, its more widespread use is impeded by the fact that its deep drawing ability is even poorer than that of the 17 percent chromium steel.

In case of high corrosive and deep drawing stresses, therefore, heretofore it has been necessary to have recourse to the austenitic chromium nickel steels. As previously mentioned, austenitic chromium nickel steels are superior to the ferritic chromium and chromium-molybdenum steels in regard to deep drawing qualities, but chromium nickel steels are substantially more expensive. In addition, there is the disadvantage of the so-called "yellowishness," so that these steels have no gained popularity for automotive parts in particular.

Austenitic types of steel have been developed to relieve the cost situation, which makes it possible to reduce the nickel content by partially replacing this element with manganese and/or nitrogen. These steels are not widely used, either, however, because they are still too expensive and the problem of "yellowishness" is still encountered in them. Examples of such steels are AISI 201 and 202.

It is known that the yield point and tensile strength can be lowered by reducing the amounts of carbon and nitrogen present ("Metallkunde," 1963, pp. 724 sqq.). This method has not become popular, either because an extensive reduction of the carbon content, such as might be expected to result in an indirect improvement in the deep drawing quality, results in an undesirable lengthening of the refining time with a resultant greater

loss of chromium, shorter furnace lining life, and the like.

A diminution of the carbon content in ferritic chromium steels by the so-called vacuum refining process is technically possible, but has not gained popularity in the manufacture of strip, since the capacities needed for this purpose are not available. Furthermore, the use of this process entails an increase in cost.

In view of the numerous and sometimes very different processes of sheet forming, it has proven to be difficult to find a universal measuring method for every possible type of cold forming. The so-called roundel ratio or maximum drawing ratio has established itself as a very meaningful index of the deep drawing ability. 15 This parameter is defined by

$$\beta = D/d.$$

In the case of cylindrical drawing, this means the ratio of the starting diameter  $D$  of the sheet steel roundel to 20 the diameter  $d$  of the finished drawn specimen ("Maschinenmarkt," Vol. 74, 1968, No. 31, p. 561). In other words, the greater the maximum drawing ratio is, the greater is the depth of the cup that is drawn. Since the roundel diameter is an indication of the roundel area 25 that is to be formed, if the roundel diameter is increased by about 10 percent, for example, about 20 percent more roundel area has to be formed, resulting in a corresponding increase in the cup depth. In practice, therefore, the object is to achieve the highest possible drawing ratios in one draw.

The maximum drawing ratio thus permits comparison of the deep drawing characteristics of various materials. Under the experimental conditions described in the literature cited above, the greatest possible roundel ratio that can be achieved in ferritic steels with their poor forming qualities is approximately 1.6 in a single draw, while the austenitic steels are much better, with values of 2.2 maximum.

It is technically possible, of course, to achieve forms by a plurality of draws, but in such cases annealing has to be performed after each draw, followed by pickling, so that there are financial limits to this procedure.

Furthermore, the loss of surface quality due to the repeated annealing would necessitate more work in finishing the workpieces.

It is obvious that, in the case of such standardized testing procedures, if the material characteristics are constant, the roundel ratio is dependent upon the shape of the punch, the radii, the drawing oil, and other such factors. In the actual comparison of various types of steel, all of the drawing conditions must, of course, be constant. The deep drawing tests herein were performed on a hydraulic drawing press with a rated capacity of 100 metric tons. A flat-faced punch was used, which had a diameter of 100 mm. The punch [edge] radius amounted to 10 mm, and the drawing die [edge] radius was 4 mm.

With this experimental set-up, maximum drawing ratios ranging from 1.96 to 2.03 for the chromium molybdenum steel X 6 CrMo 17, were obtained while chromium nickel steel produced ratios of 2.16 to 2.25. As already explained, this is a considerable difference because, under these conditions, chromium nickel steels permit the forming of an approximately 20 percent greater roundel surface without cracking; consequently substantially deeper cups can be drawn than with chromium steel. It is known, therefore, that the deep draw-

ing of ferritic steels involves an appreciable expenditure on multiple draws, annealing between draws, and surface finishing operations, since, in many cases, chromium nickel steels cannot be substituted for the reasons given earlier.

### SUMMARY

The present invention involves a new process whereby the deep drawing ability of ferritic chromium steels containing molybdenum is so substantially improved that it is similar to the austenitic chromium nickel steels. That the field of application of this type of steel is thus substantially expanded.

The improvement in deep drawing qualities is brought about by, according to the invention, by the application of the following steps:

a. For the manufacture of the strips and sheets according to this invention the following steel composition is used, containing:

0.005 — 0.12% carbon

0 — 1.0% silicon

0.3 — 3.0% manganese

15.0 — 20.0% chromium

0.15 — 3.0% nickel

0.5 — 1.5% molybdenum

0.05 — 0.20% nitrogen

0 — 0.10% aluminum

Balance: iron and impurities,

and this composition gives an F factor of 3.3 to 6.0 if the following equation is applied:

$$F = [80 (\%C) + 1300 (\%N) + 150 (\%Ni) + 25 (\%Mn) + 8 (\%Cu)]/[3.6 (\%Cr) + 9 (\%Si) + 7.6 (\%Mo) + 75 (\%Al)]$$

b. These steels are subjected, in the form of the hot-rolled strip, to a multi-stage box annealing in the range of 970° to 600°C, the temperature being lowered step-wise by at least 30°C in each step, and

c. Annealing is performed between the individual cold rolling steps and after the final step at temperatures of 820° to 650°C, with holding times of 5 seconds to 10 minutes, followed by cooling.

All percentages given herein are by weight unless indicated otherwise.

### DESCRIPTION

Extensive experiments have shown that the steel composition used in this invention in conjunction with special annealing measures in the hot-rolled state and during the cold working process make possible a great improvement over the art as regards the deep drawing capacity of this type of steel.

The steel composition used in this invention comes partially within the scope of the molybdenum alloy — 17 percent chromium steels of the following composition:

C 0.005 — 0.12%

Si 0.2 — 0.6%

Mn 0.2 — 0.6%

Cr Approx. 17%

Mo Approx. 1.0%

The standards for this type of steel composition varies as follows:

German Preliminary Standard DIN 17440:

C ≤ 0.07%

Si ≤ 1.0%

Mn ≤ 1.0%

Cr 16.0 — 17.5%

Mo 0.9 — 1.2%  
Balance: iron and impurities.  
USA Standard A.I.S.I. Type 434:

C ≤ 0.12%

Si ≤ 1.0%

Mn ≤ 1.0%

Cr 16.0 — 18.0%

Mo 0.75 — 1.25%

Bal.: iron and impurities.

10 Known chromium steels contain, in their regular commercial form, a maximum of about 0.30% nickel, about 0.03% nitrogen, and a maximum of 0.20% copper. The aluminum content runs up to 0.05%. On the basis of these common alloying admixtures, factors of F ≤ 2.5 are obtained when the above equation is applied.

15 However, it is necessary according to this invention to achieve F values of 3.3 to 6.0. This is achieved by increasing the normal contents of carbon, nickel, manganese, copper, and especially nitrogen used in alloying

20 such steels. The decided improvement in deep drawing qualities which is achieved by this in combination with the other two measures described herein is unexpected. Whereas the state of the art teaches improving deep drawing qualities by diminishing the amounts of carbon

25 and nitrogen present, an impressive improvement over the prior-art figures is achieved unexpectedly by increasing the quantity certain components previously thought to be harmful, and by the simultaneous application of the two special annealing measures described 30 herein.

According one embodiment of the process, it is advantageous if the F factor computed according to the above equation equals 3.4 to 5.3. It is furthermore advantageous to select the alloy composition such that F is between 3.5 and 4.5, and preferably between 3.7 and 4.3.

35 The box annealing of hot rolled strips and sheets of chromium steels and chromium molybdenum steels, which is designed to eliminate the linear arrangement 40 of the ferrite grains and carbides produced as a result of the preceding hot rolling process, it customarily performed under inert gas in the 850° to 800°C range ("Bander — Bleche — Rohre," Duesseldorf, 2, 1963, p.61). The box annealing of hot rolled strip is normally 45 performed in one step. Multi-step annealing processes can be used if desired.

A multi-step hot rolled strip annealing process for ferritic chromium steels prevents the occurrence of the so-called "riffle structure" and improves the 50 mechanical-technological characteristics (German Auslegeschrift No. 1,222,520).

The solution of the problem to which the invention is addressed is achieved by the precise selection of the 55 steel composition through the alloying quotients and the simultaneous use of stepped box annealing of the hot rolled strip and intermediate annealing after one of the cold-rolling steps in some cases and, in any case, final annealing after the last cold-rolling step.

60 The possibility of raising the β value in 17% chromium steels above the normal level has not previously been possible.

In a number of publications other multiple annealing processes have become known, which are intended to 65 eliminate the linear arrangement of the hot-rolled strip structure in ferritic chromium steel to which no molybdenum is added. This improvement is achieved by a more or less long annealing of the hot-rolled strip, pref-

erably in a temperature range between 950° and 1,100°C, followed by cooling to room temperature, and followed again by annealing in the temperature range of around 805°C which is customary for ferritic chromium steels. The publications in question are U.S. Pat. Nos. 2,772,992, 2,808,353 and 3,139,358. From these patents is it not possible to learn how the  $\beta$  value can be raised above the normal level in the case of 17% chromium molybdenum steels.

The multi-step hot-rolled strip annealing prescribed according to the invention, in the form of three-step annealing, consists of the following process steps:

1. Annealing for 30 min to 15 hours at 970° – 800°C.
2. Cooling in furnace by at least 30°C to a temperature of 850° – 600°C.
3. Annealing of 5 to 40 hours at 850° to 600°C.

The preferred temperatures are 920° – 850°C for the first process step, and 740° – 650°C for the third step. According to an additional embodiment of the invention, the multi-step hot-rolled strip annealing can consist of a continuous five-step treating process entailing the following steps:

1. Annealing for 30 min to 15 hours at 970° – 800°C.
2. Cooling in furnace by about 30°C to a temperature of 850° – 700°C.
3. Annealing for 1 to 40 hours at 850° – 700°C.
4. Furnace cooling by at least 30°C to a temperature of 750° – 600°C.
5. Annealing for 5 to 40 hours at 850° – 600°C.

The annealing in this embodiment of the process is preferably between 920° and 850°C for the first step, between 800° and 720°C for the third step, and between 730° and 650°C for the fifth step.

In addition to the three-step and five-step annealing processes described in detail above, other hot-rolled strip annealing processes involving greater numbers of steps come within the scope of the teaching of the invention. Nevertheless, the upper limit of 970°C, the minimum of 30°C for each step in the temperature reduction, and the lower temperature limit of 600°C must be observed.

These measures are novel for 17% chromium molybdenum steels and so advantageous in their effect that the longer box annealing time is amply compensated.

The annealed and pickled hot-rolled strip can be cold-rolled by known methods.

Cold-rolling hardens the chromium molybdenum steel and therefore it has to be annealed prior to cold forming or deep drawing operations. The technical expert is familiar with the fact that higher temperatures result in better ductility in the finished strips, but loss of surface quality places limits on the temperature that can be used. Temperatures of 850°C are rarely exceeded. To protect the surface the steel strips are annealed in a continuous furnace and then pickled in chemical baths.

Since relatively high strip speeds must be used for reasons of output and cost (e.g., at a strip thickness of 1 mm and a furnace length of about 30 m, the speed is greater than 15 m/min, resulting in an annealing time of 18 sec), the temperature has to be raised faster and the holding time has to be shortened accordingly in order to assure perfect annealing. Usually, therefore, short periods are sufficient, depending on the strip thickness, to transform the strip to a ductile state, although in the case of chromium molybdenum steels temperatures of 850° – 820°C are necessary in order to

achieve the state of optimum formability at short annealing times (e.g., max. 10 min for a strip 5 mm thick).

Surprisingly, the process of the invention succeeds with substantially lower temperatures. Contrary to the technical teaching that has been known and described above, this steel has to be annealed at temperatures of 780° to 700°C in order to have the maximum ductility and outstanding deep-drawing characteristics.

An additional embodiment of the process calls for a preferred annealing range of 770° – 720°C. Temperatures of 750° – 730°C are also possible. It is sufficient that the strip be held at these temperatures for 5 seconds to 10 minutes. It is therefore advantageous to perform this annealing in continuous furnace, although stationary annealing process can also be used.

It is surprising in this invention that, in spite of the fact that it runs counter to known procedures and results in several respects, it results in an improvement in deep drawing characteristics that goes beyond the state of the art. This involves especially in alloying the elements carbon and nitrogen, and in the appreciable lowering of the intermediate and/or final annealing temperatures below the customary levels.

Nevertheless, the combination of these measures with the special box annealing process produces a new effect, which consists in an improvement of deep drawing ability in 17% chromium molybdenum steels to an extent unknown hitherto.

The improvement in deep drawing properties is also produced when the final annealing is performed such that 1 to 10% transformation structures are present in addition to ferrite in the finished strip. This effect, with which the technical expert is familiar, is known to occur when steels having a  $\gamma$  to 60 transformation are heated so high and so long that the  $\gamma$  region is present at least partially, and are then cooled in such a manner that the state of equilibrium in the structure is fore stalled.

This individual measure is described in a similar manner in German Pat. No. 1,188,109, and serves in that patent to eliminate the so-called "flow lines sensitivity." Whereas it is necessary in this patent to operate with relatively high temperatures, the combination of the intermediate and/or final annealing (according to German Pat. No. 1,188,109) with the present invention has the advantage that the effect of the elimination of low figures occurs at temperatures as low as the lower limit or below the customary final annealing temperature. In addition, a further improvement of the deep drawing qualities is possible. And furthermore, the dressing operation is eliminated which is normally necessary in the production of ferritic chromium molybdenum steels and this has a very noticeable positive effect as regards costs, since this dressing operation requires special rolling trains equipped with rolling and grinding devices and the like.

With the process of the invention it is possible to produce ferritic chromium molybdenum steels whose deep-drawing characteristics are comparable to the substantially more expensive austenitic chromium nickel steels. Using the experimental deep-drawing press described above, it has been possible easily to achieve maximum drawing ratios of approximately 2.25 with numerous strips and sheets manufactured according to the invention.

The invention is further described in the following examples:

## CONTROL 1

## The Prior Art

A melt of the following chemical composition:

|                         |
|-------------------------|
| C — 0.05%               |
| Si — 0.40%              |
| Mn — 0.40%              |
| Al — 0.03%              |
| Ni — 0.20%              |
| Cr — 17.1%              |
| Cu — 0.12%              |
| Mo — 1.0%               |
| N <sub>2</sub> — 0.031% |

was prepared in an electric furnace, cast into slabs, and rolled in a roughing mill to a strip 4 mm thick.

The application of the formula given above showed the F factor to be 1.136. The hot-rolled strips were annealed in a stack in the box annealing furnace for a period of 34 hours at 840°C, then pickled, and then cold-rolled to 1.5 mm thickness. Then the material was annealed at 840°C for about 20 sec and pickled. Afterward, the strips were rolled again to a final thickness of 0.6 mm, treated for about 15 sec at 850°C in the continuous annealing furnace and then pickled. After the continuous annealing process the strips were sensitive, in intermediate and final thickness, to the occurrence of the flaw known as "flow figures." The material therefore had to be re-rolled twice in final thickness in a dressing machine.

Flow-figure susceptibility was found to be absent in the final examination for release. A deep drawing test of the material on the press described above produced  $\beta$  values of 2.0 in the 1.5 mm thickness, and in the finished state the maximum drawing ratio was  $\beta = 2.02$ .

Another pickled hot-rolled strip from the same melt was cold-rolled to 0.6 mm without any intermediate annealing treatment, then annealed for 15 sec at 850°C and pickled. On account of its susceptibility to flow figures, this strip also had to be dressed in two passes, and in the finished state it had a maximum drawing ratio  $\beta = 2.03$

## CONTROL 1

## The Invention

A melt of the following composition:

|                         |
|-------------------------|
| C — 0.07%               |
| Al — 0.004%             |
| Ni — 0.71%              |
| Si — 0.22%              |
| Cr — 16.15%             |
| Cu — 0.24%              |
| Mn — 1.45%              |
| Mo — 0.87%              |
| N <sub>2</sub> — 0.096% |

was rolled, as in control 1, to 4 hot-rolled strips of a thickness of 4 mm. The use of the equation showed an F factor of 4.103. Two sets of two each of these hot-rolled strips were subjected to a three-step box annealing procedure as follows:

Run 2.1: The strips were annealed for 3 hours at 880°C, then cooled in the furnace by 170°C to 710°C and held at this temperature for 20 hours.

The total annealing time amounted to 41 hours.

Two more sets of two hot-rolled strips from the same melt were treated by a five-step box annealing procedure as follows:

Run 2.2: These strips were annealed for 2.5 hours at 900°C; after furnace cooling by 160°C down to 740°C they were held at the latter temperature for 6 hours, furnace-cooled again by 40°C down to 700°C and held at this temperature for 15 hours. The total annealing time was 43 hours.

All of the hot-rolled strips were pickled. One strip 2.11 and strip 2.21 were cold rolled to 1.5 mm thickness and, in the roll-hard state, they were divided into two halves. The one half 2.111 and 2.211 was annealed for about 20 sec at 760°C, then rolled down to a final thickness of 0.6 mm and divided into two halves.

The second hot-rolled strip 2.12 and 2.22 was cold-rolled directly to 0.6 mm and also divided into two strips while in the roll-hard state. The one half of the cold-rolled strip in each case, in the 0.6 mm thickness, was given a final annealing for about 15 sec at 760°C. Examination of the material in the finished state showed a ferritic structure and flow-figure susceptibility in all strips of the 1.5 and 0.6 mm thicknesses. The finished strips therefore had to be dressed in two passes. Then the flow-figure susceptibility was eliminated.

Testing for deep drawing ability showed maximum draw ratios  $\beta$  between 2.21 and 2.23 for the strips in the 1.5 mm thickness. In all of the finished strips of the 0.6 mm thickness, maximum draw ratios  $\beta$  of 2.24 to 2.26 were found after direct rolling and also after two-step rolling through the intermediate thickness.

The strip halves in the intermediate and final thicknesses which had been cut in the roll-hard state, Nos. 2.112, 2.12, and 2.122, 2.222, 2.1112 and 2.2112, were subjected to another separate annealing. The strips 2.112 and 2.212 of the 1.5 mm thickness were annealed 25 sec at 810°C and cold-rolled to 0.6 mm; all strips of the 0.6 mm thickness were treated at 810°C in the continuous annealing furnace and force-cooled. After pickling, all of the strips in the finished state showed transformation structure along with 3 to 6% ferrite. All strips were free of flow figures and therefore they could be cut into plates and shipped to fabricators without any additional dressing procedure. In this state, maximum draw ratios  $\beta$  of 2.24 to 2.27 were found.

## EXAMPLE 2

## The Invention

A melt of the chemical composition

|                        |
|------------------------|
| C — 0.07%              |
| Al — 0.002%            |
| Ni — 1.0%              |
| Si — 0.18%             |
| Cr — 16.08%            |
| Cu — 0.26%             |
| Mn — 1.60%             |
| Mo — 0.85%             |
| N <sub>2</sub> — 0.06% |

was made, as described in Example 1, into cold-rolled strip of the 0.6 mm thickness, some of it through the 1.5 mm intermediate thickness and some of it by direct rolling. The alloying quotient (F) of this melt was 4.169. In the case of the separate final annealing and forced cooling which was used in part, the making of this melt into cold-rolled strip differed only in that, to eliminate the dressing procedure, the strips were annealed at a temperature of 800°C with the same holding times as in Example 1, and after this separate annealing

and forced cooling they were found to have 3 to 5% transformation structure.

The rest of the strips or portions of strip prepared according to the invention, which had been treated to create transformation structure, were subjected according to the invention to a final annealing in the 730°-740°C range, cooled normally, and were ferritic as well as susceptible to flow-figure formation, so that they then had to be dressed.

What is claimed is:

1. Process for the manufacture of cold-rolled strips and sheets from corrosion-resistant ferritic chromium steel with molybdenum added which comprises forming a hot-rolled strip from an alloy having the composition:

0.005-0.12% — Carbon

0-1.0% — Silicon

0.3-3.0% — Manganese

15.0-20% — Chromium

0.15-3.0% — Nickel

0.5-1.5% — Molybdenum

0.05-0.20% — Nitrogen

0-0.50% — Copper

0-0.10% — Aluminum

Balance: iron and impurities,

said alloy having an F factor equal to 3.3 - 6.0 calculated using the equation

$$F = [80 (\%C) + 1300 (\%N) + 150 (\%Ni) + 25 (\%Mn) + 8 (\%Cu)]/[3.6 (\%Cr) + 9 (\%Si) + 7.6 (\%Mo) + 75 (\%Al)]$$

annealing the hot-rolled strip in a plurality of steps below 970°C and above 600°C, the temperature being lowered step-wise but at least 30°C during each annealing step, cold-rolling said strip and after each cold-rolling step, annealing at temperatures of 820 - 650°C and at holding time of 5 sec to 10 min. and cooling the annealed material.

2. Process of claim 1, wherein said alloy has an F factor between 3.4 and 5.3.

3. Process of claim 1, wherein said alloy has an F factor between 3.5 and 4.5.

4. Process of claim 1, wherein said alloy has an F fac-

tor between 3.7 and 4.3.

5. Process of claim 1, wherein before cold rolling a three-step annealing process consisting of the following steps is carried out:

- 5 a. Annealing for 30 min to 15 hours at 970°-800°C.
- b. Cooling by at least 30°C to a temperature of 850° - 600°C.
- c. Annealing for 5 to 40 hours at 850° - 600°C.

- 6. Process of claim 5, wherein step (a) is carried out at a temperature between 850° and 920°C. and step (c) is carried out at temperatures between 740° and 650°C.

7. Process of claim 1, wherein before cold rolling a five-step hot-rolled strip annealing process consisting of the following steps is carried out:

- 15 a. Annealing for 30 min to 15 hours at 970° - 800°C.
- b. Cooling by at least 30°C to a temperature of 850° - 700°C.
- c. Annealing for 1 to 40 hours at 850° - 700°C.
- d. Cooling by at least 30°C to a temperature of 750° - 600°C.

- e. Annealing for 5 to 40 hours at 750° - 600°C.

8. Process of claim 7, wherein step (a) is carried out at temperatures between 920° and 850°C, step (c) is carried out at temperatures between 800 and 720°C,

25 and step (e) is carried out at temperatures between 730° and 650°C.

9. Process of claim 1, wherein annealing after at least one cold-rolling step is carried out at a temperature between 780° and 700°C.

10. Process of claim 9, wherein the annealing is carried out at a temperature between 770° and 720°C.

11. Process of claim 9, wherein the annealing is carried out at a temperature between 750° and 730°C.

12. Process of claim 1, wherein characterized the annealing after at least one cold-rolling step is held in the 820°-650°C range for a period of time and is cooled in a manner such that after cooling, 1-10% transformation structure is present in the end product.

13. Process of claim 1, wherein the annealing after at least one cold-rolling step is carried out in continuous furnaces after at least one cold-rolling pass.

\* \* \* \* \*